

June 5, 1945.

J. V. FILL

2,377,486

METHOD AND APPARATUS FOR MAKING CARBONYL IRON

Filed May 22, 1941

*Fig. 1.*



*Fig. 2.*



*Fig. 3.*



INVENTOR  
*JOHN V. FILL*  
BY  
*Bernard Wilson F. Gammie*  
ATTORNEYS

## UNITED STATES PATENT OFFICE

2,377,486

METHOD AND APPARATUS FOR MAKING  
CARBONYL IRONJohn V. Fill, Dobbs Ferry, N. Y., assignor to Micro  
Products Corporation, Dover, Del., a corpora-  
tion of Delaware

Application May 22, 1941, Serial No. 394,656

4 Claims. (Cl. 75—33)

This invention relates to a method and apparatus for making carbonyl iron for use in magnetic cores for radio apparatus and the like.

The extremely minute particles of iron which are deposited in the thermal decomposition of ferro-pentacarbonyl have proved highly desirable for use in making magnetic cores. In order to be most perfectly adapted for this purpose the minute iron particles should consist of spherical shells of decreasing thickness.

I found that the form of the iron particles depends upon the pressure and concentration of the iron carbonyl gas during the decomposition thereof and that to obtain the particles in the best possible form the pressure and concentration of the carbonyl gas should be reduced during the decomposition. This results in causing the iron to deposit in layers on nuclei which are formed when the gas is at high pressure and concentration. The layers become thinner as 20 the concentration and pressure decrease.

My invention provides a continuous method of decomposing iron carbonyl under conditions of decreasing pressure and decreasing concentration. This is accomplished in accordance with the invention by introducing compressed gaseous ferro-pentacarbonyl into the upper part of a tapering chamber. The decomposition occurs as 25 the gas and the deposited particles move downwardly in the chamber. In this downward movement the concentration and pressure of the gas decrease with the evolution of carbon monoxide gas and the increase in the cross section of the chamber.

In order that my invention may be clearly understood, I will describe in detail a method embodying the invention carried out in the apparatus embodying the invention which is shown in the accompanying drawing in which,

Fig. 1 is a sectional elevation of the apparatus in the form which I consider most desirable; and

Figs. 2 and 3 are diagrammatic sectional elevations showing modified forms of the apparatus.

The apparatus shown in Fig. 1 includes an inner funnel-shaped or conical chamber 2 with its larger end directed upward, and an outer annular frusto-conical chamber 4 with its larger end directed downward. A baffle 3 is provided for directing gas from the larger end of the inner chamber into the smaller end of the outer chamber. Vertical pipes 9 extend from outlet openings in the bottom of the outer chamber 4 to collectors 10 provided with gas vents 12. The inner chamber 4 is provided with a heating jacket 5, 55

and the pipes 9 may be provided with cooling coils 11. An inlet pipe 1 is connected to the lower end of the inner chamber 2.

In carrying out my method my means of this apparatus a high temperature is maintained in the chambers 2 and 4, and liquid ferro-pentacarbonyl is introduced into the inner chamber 2 through the pipe 1 at such a rate that the liquid is converted into a gas but is not decomposed 10 as it rises through the inner chamber 2. The volatilization of the liquid creates pressure so that gaseous carbonyl under considerable pressure enters the upper end of the outer chamber 4. As the carbonyl gas descends in the chamber 15 4 it decomposes into iron and carbon monoxide gas. Because of the diverging walls of the chamber 4 the carbonyl is decomposed under conditions of decreasing pressure and decreasing concentration so that the iron is deposited in thinner and thinner layers on the nuclei which have formed at or near the top of the chamber 4.

The iron particles formed in the chamber 4 fall through the pipes 9 into the collectors 10. The carbon monoxide gas formed in the decomposition, whose volume is somewhat reduced by the cooling coils 11, passes into the collectors 10 and out through the pipes 12 whence it may be conducted to an apparatus for making ferro-pentacarbonyl.

The temperature in the chamber 4 is indicated by thermo-couple 8. Supply of heating medium to the jacket is most desirably regulated so as to maintain the temperature in the chamber 4 at approximately 200° F.

It is not essential that the carbonyl move upwardly while it is being converted into a gas. Thus, while the apparatus which has been shown in Fig. 1 is compact and convenient it may be modified by inverting the inner chamber 2 and placing it on top of the outer chamber 4 so that the two chambers become a single conical chamber with its larger end downward, as shown in Fig. 2. The chamber may be in the form of a prism instead of a cone, or may take the form of an ellipsoid of revolution, as shown in Fig. 3.

What I claim is:

1. The method of making carbonyl iron which consists in thermal decomposition of ferro-pentacarbonyl under conditions of increasing volume, decreasing concentration and decreasing pressure.

2. The method of making carbonyl iron which consists in causing compressed ferro-pentacarbonyl gas to move downwardly in a heated chamber whose walls diverge so that the hori-

zontal cross section of the chamber increases downwardly, so that thermal decomposition of the ferro-carbonyl occurs under conditions of decreasing concentration and decreasing pressure.

3. Apparatus for making carbonyl iron comprising a chamber having diverging walls so that its horizontal cross section is largest at its lower end, collectors connected to the bottom of the chamber, means for introducing compressed gas at the upper part of the chamber, means for heating the chamber, and cooling means located between the chamber and collectors.

4. Apparatus for making carbonyl iron comprising an inner conical chamber with its larger end upward and an outer conical chamber with its larger end downward, baffles for directing gas from the larger end of the inner chamber into the smaller end of the outer chamber, an inlet pipe at the smaller end of the inner chamber, outlet pipes at the larger end of the outer chamber and a heating jacket around the outer chamber.

JOHN V. FILL.